# EUROPEAN PATENT APPLICATION

(11) **EP 2 037 022 A2**
(43) Date of publication of application: **18.03.2009**
(21) Application number: 08163846.2
(22) Date of filing: 08.09.2008
(51) Int. Cl.: D03D 15/02, D03D 15/04

(54) **Tire cord fabric**

(30) Priority: 14.09.2007 US 855253
(71) Applicant: The Goodyear Tire & Rubber Company, Akron, OH 44316-0001 (US)
(72) Inventor: Conger, Kenneth Dean, Stow, OH 44224 (US); Kot, Kenneth Michael, Canton, OH 44708 (US); Madaras, Jon Michael, Fairlawn, OH 44333 (US); Bujak, Paul Michael, Cuyahoga Falls, OH 44223 (US)
(74) Representative: Kutsch, Bernd

(57) **Abstract**

A tire cord fabric (10) is provided that has a first portion and a second portion. The tire cord fabric comprises warp cords (12) oriented in the longitudinal direction and weft yarns (14) oriented in the lateral direction. The warp cords are used in reinforcing pneumatic tires. In the second portion, the weft yarns (18) have an increased count per inch versus the count per inch of the weft yarns (14) in the first portion of the fabric (10). The weft yarns in the second portion (16) are preshrunk prior to weaving of the tire cord fabric.

## Description

### Field of the Invention

The present invention is directed to a tire cord fabric and to a method of manufacturing tire cord fabric and the type of yarn used in the end, or tabby portions, of tire cord fabric.

### Background of the Invention

Fabric used in the reinforcing of tires normally comprises tire cords placed in the warp or longitudinal direction of the fabric, with the warp tire cords being woven or held by a relatively weak weft yarn oriented perpendicular to the cords. The number of tire cords per inch in tire cord fabrics normally varies depending on the end uses and the tire specification. The number of weft yarns per inch also varies.

The weft yarns serve the purposes of maintaining the structural integrity of the fabric during further fabric treatment and maintaining the desired spacing between the warp tire cords during building and expansion of the green tire.

It is a common practice to treat tire reinforcing fabric with liquid adhesives. This treatment is to improve the adhesion between the fabric and the rubber matrix of the tire. The untreated fabric is normally wound into a roll. As the last piece of fabric leaves the roll and before it enters the dip unit, the tail end of the roll is attached to the first end of the next roll to be treated. Where the ends of the rolls are to be attached together, the count per inch of the weft yarn is increased at the end of the roll to contribute to the strength of the splice or seam. This increased count per inch weft yarn area of the fabric is known as the tabby and normally measures in length between 5 and 20 inches. The tabby is not used in reinforcing tires and is discarded as waste at some point in the rubber calendering operation.

Because of the closeness of the weft yarns to one another in the tabby section of the fabric, there is an increased crimping of the weft yarns by the warp cord, which is held under tension during the weaving. This leads to a narrowing of the fabric width to accommodate the increased count per inch of weft yarn, transforming the ends of the fabric from a relatively straight configuration to a wavy or crimped configuration. Additionally, during heat treatment of the fabric, shrinkage of the weft yarns can cause the tabby to further contract, see FIG. 2. The narrowing of the tabby can result in wrinkling of the fabric and inconsistent dipping of the fabric during treatment.

While it has been accepted that the tabby portion is discarded as waste during calendering, due to the narrowing of the tabby fabric during conventional treatment, a portion of the regular tire cord fabric is also reduced in width, FIG 2, and is discarded along with the tabby area, resulting in increased waste. Also, this narrowing of the tabby results in disturbances in the process, especially with the fabric spreading and guiding equipment. These disturbances result in waste due to poor warp cord quality near the tabby, poor wind-up quality, fabric web splits, etc.

### Definitions

Tabby means a portion of a fabric having increased weft yarn counts per inch versus the weft yarn counts per inch of a main portion of said fabric. Preferably, the tabby is located at the end of a piece of fabric when rolled up on a roll.

### Summary of the Invention

The present invention is directed to a tire cord fabric and a method of producing tire cord fabric according to claims 1 and 10 respectively having an improved structure for a tabby for instance wherein width reduction of the tabby and the adjacent fabric portion are reduced, thereby reducing waste and improving fabric treatment consistency.

Dependent claims refer to preferred embodiments of the invention.

### Brief Description of the Drawings

The invention will be described by way of example and with reference to the accompanying drawings in which:
FIG. 1 illustrates a tire cord fabric; and
FIG. 2 illustrates a prior art tire cord fabric after treatment.

### Detailed Description of the Invention

In FIG. 1, a fabric 10 is illustrated. The fabric 10 is formed of a plurality of warp cords 12 and weft yarns 14. In the main portion of the fabric 10, typically comprising more than 98%, preferably 99% or more of the length of the fabric 10, the weft yarns 14 are generously spaced from one another at a count per inch of 0.5 to 3 per inch (1.3 to 7.6 per cm). At the terminal end of the fabric 10, the density of the weft yarns 14 is increased to form a tabby 16. Hence, the length of the tabby is less than 2%, preferably 1% or less, of the length of the fabric 10.

The warp cords 12 are tire cords and may be formed from any materials used for tire cords, including, but not limited to, steel, carbon fiber, aramid, nylon, rayon, polyester, fiberglass, polyvinyl alcohol, or any blends thereof, or other future types of tire cords. The exact cord specifications and the spacing of the warp cords are determined by the tire specification.

As the weft yarns 14 function primarily to maintain the spacing of the warp cords 12 in the main portion of the fabric 10, the diameter, denier, and/or strength of the weft yarns 14 need not be equal to that of the warp cords 12. The weft yarns 14 are generally selected from any suitable material having a breaking strength of preferably from 1.5 to 4 pounds (0.68 to 1.81 kg), and an elongation at break of preferably from 20 to 45 percent. The size of the weft yarn 14 depends on the corresponding size of the warp cord 12. The weft yarns 14 are generally selected from lightweight materials such as polyester, cotton, rayon, nylon, or blends thereof.

In the tabby 16, to provide strength assistance in the splice or seam when joining fabric rolls/lengths, the weft yarns 18 of the tabby 16 may be different than the weft yarns 14 in the main portion of the fabric 10. The tabby weft yarns 18 may be selected from the same material, with an increased denier to provide a denser, stronger yarn, or may be selected from an entirely different material with different yarn specifications.

In a conventional fabric 100, when the fabric 100 is treated, as discussed above, the tabby 102 is reduced in lateral width due to shrinkage and crimping of the tabby weft yarns 104. However, the width reduction is not limited to the tabby 102 and a portion 106 of the fabric 100 also has reduced lateral width and this portion 106 of the fabric 100 is generally relegated to waste material. While FIG. 2 is purely illustrative of the lateral shrinkage, the fabric 100 has an approximately 37.5% loss in width due to shrinkage and at least a 10% loss in width is conventional.

In accordance with the goal of the present invention - to reduce the lateral width shrinkage of the tabby 16 as the fabric 10 is treated, the tabby weft yarns 18 are selected for reduced shrinkage. Any conventional tabby weft yarn may be used; however, the yarn, prior to being woven into the tabby 16, must be preshrunk or be made of a preshrunk material. Preshrunk means that the yarn is processed by treatment so that its length is not reduced by more than 1 to 10 percent, more particularly, only by 1 to 3 percent or less during a fabric treatment or an other processing step after the treatment to reduce shrinkage of the yarn. Preferably, the yarn is preshrunk so that its length is not reduced by more than 1% during a fabric treatment such as heat treatment and/or a treatment with liquid adhesives in a dip unit. Specific preshrinking treatment will be dependent upon the type of yarn, but may comprise for example, a two zone process. In the first zone, the material may be over stretched at a tension ranging from 10% to 25% of the greige cord's breaking strength. In the second zone, the material may be relaxed wherein the tension is less than 5% of the greige cord breaking strength. The temperatures for both zones may be in the range of 90% to 97% of the material's melting point. For a cotton weft yarn, preshrinking typically may include exposure to high heat in a humid condition such as a hot water bath and drying.

Conventionally, both weft 14 and tabby weft 18 yarns are not preshrunk prior to use in tire cord weaving operations. Instead, yarn is used directly from the yarn manufacturer, and all treatment of the yarns 14, 18 occurs with the treatment of the fabric. By using preshrunk yarn as the tabby weft 18, the width reduction in the tabby 16 is reduced and any portion of the fabric 10 that is also reduced due to the tabby width reduction is minimized, thereby reducing waste and improving adhesive treatment of the fabric. There may continue to be a loss of width in the tabby 16 due to crimping; however, this loss should be limited to less than 5% of the fabric width; the tabby 16 should have a width of at least 95% of the width of the main fabric portion.

The tabby weft yarns 18 of the present invention can be used in the body of the fabric, as well as the tabby 16. Where the body of fabric is subject to severe thermal shrinkage conditions and mechanical tensioning such that the combination of factors results in unreasonable width reduction in the body of the fabric 10, the use of the tabby weft yarn 18 of the present invention in the body of the fabric is beneficial.

## Claims

1. A tire cord fabric having a longitudinal direction, a lateral direction, a first portion and a second portion, the tire cord fabric comprising warp cords (12) oriented in the longitudinal direction and weft yarns (14) oriented in the lateral direction, the warp cords (12) being tire cords, wherein the weft yarns (18) in the second portion have an increased count per inch versus the count per inch of the weft yarns (14) in the first portion of the fabric (10), **characterized in that** the weft yarns (18) in the second portion are preshrunk prior to weaving of the tire cord fabric and/or are made of a material that provides that the length of the weft yarns in the second portion is not reduced by more than 10 percent in a tire cord fabric treatment.

2. The tire cord fabric of claim 1 wherein the preshrunk weft yarns in the second portion or the material of the weft yarns in the second portion have a remaining shrinkage of not more than 1 % of the length of the weft yarn.

3. The tire cord fabric of claim 1 wherein the preshrunk weft yarns in the second portion or the material of the weft yarns in the second portion from claim 2 have a remaining shrinkage of 1 % to 3% of the length of the weft yarn.

4. The tire cord fabric of at least one of the previous claims wherein the first portion is a main portion of the fabric (10) and wherein the second portion is a tabby (16).

5. The tire cord fabric of claim 4 wherein the tabby (16) has the same or a reduced lateral width in comparison to the main portion, the tabby (16) having a width of at least 99% of the width of the main portion.

6. The tire cord fabric of at least one of the previous claims wherein the fabric (10) is adhesively treated.

7. The tire cord fabric of at least one of the previous claims wherein the weft yarns (14) in the main portion or in the first portion are also preshrunk.

8. The tire cord fabric of at least one of the previous claims wherein the material of the preshrunk weft yarns (18) is selected from the group consisting of polyester, cotton, rayon, nylon, or blends thereof.

9. The tire cord fabric of at least one of the previous claims wherein the main portion is at least 98%, alternatively at least 99%, of the length of the fabric (10).

10. A method of manufacturing a tire cord fabric (10) having a longitudinal direction, a lateral direction, a first portion and a second portion, the tire cord fabric comprising warp cords (12) oriented in the longitudinal direction and weft yarns (14) oriented in the lateral direction, the warp cords (12) being tire cords, wherein in the second portion the weft yarns (18) have an increased count per inch versus the count per inch of the weft yarns (14) in the first portion of the fabric (10), the method comprising preshrinking the weft yarns (14) to be used in the second portion prior to incorporating them into the tire cord fabric (10) in the second portion.

11. The method of claim 10 wherein the weft yarns (18) are preshrunk so that their length is not reduced by more than 3%, alternatively not more than 1%, during a fabric treatment such as a liquid adhesive treatment in a dip unit and/or a heat treatment.

12. The method of claim 9 or 10 wherein the preshrinking comprises a two zone process comprising an over stretching and a relaxing.

13. The method of claim 12 wherein the over stretching is done at a tension ranging from 10% to 25% of the greige cord's breaking strength and wherein the relaxing is done at a tension of less than 5% of the greige cord's breaking strength.

14. The method of at least one of the previous claims wherein the first portion is a main portion and the second portion is a tabby (16) of the fabric (10).
